

## 1

2,726,954

## TITANIUM BASE ALLOY

Robert I. Jaffee and Horace R. Ogden, Columbus, Ohio, assignors, by mesne assignments, to Rem-Cru Titanium, Inc., Midland, Pa., a corporation of Pennsylvania

No Drawing. Application October 20, 1949,  
Serial No. 122,576

11 Claims. (Cl. 75—175.5)

This invention relates to novel titanium-base alloys having properties which render the alloys highly useful for structural purposes.

In a companion application, Serial Number 122,577, filed October 20, 1949, now Patent No. 2,554,031, granted May 22, 1951, the present inventors have disclosed certain structural alloys which include the addition of a few percent of molybdenum to a titanium-base alloy containing from about 2% to about 8% of aluminum.

tween 0.1% and 0.3% of carbon, with or without 0.01% to 0.15% nitrogen or 0.01% to 0.25% oxygen, or both oxygen and nitrogen, is generally quite beneficial. Among the alloys of this invention are those made either 5 with a commercial titanium base meeting such specifications, or with a high purity titanium base containing similar amounts of added carbon, oxygen and/or nitrogen. Thus, within the purview of the invention are ternary alloys containing from about 2% to about 7% aluminum and up to about 15% chromium, as additions to a 10 titanium-base which may be of high purity or may contain up to 0.15% nitrogen, 0.25% oxygen and/or 0.3% carbon; the total nitrogen, oxygen and carbon content preferably not exceeding 0.5%. Also within the purview of 15 the invention are quaternary alloys containing up to about 5% aluminum, up to 1.25% chromium, and up to 1.25% molybdenum, as additions to the same titanium bases.

The physical properties of illustrative ternary alloys based on high purity titanium with various additions of 20 carbon, oxygen and/or nitrogen, as hot rolled and annealed at 850° C., are given in the table below, in which the proportional limit, yield strengths and ultimate strength are in units of thousands of pounds per square inch.

| Composition, Ti Base    | Al | Cr   | Tensile Properties |             |             |             |          |                          |                        |
|-------------------------|----|------|--------------------|-------------|-------------|-------------|----------|--------------------------|------------------------|
|                         |    |      | Vickers Hardness   | Prop. Limit | 0.1% Offset | 0.2% Offset | Ultimate | Percent Elongation in 1" | Percent Area Reduction |
|                         |    |      |                    |             |             |             |          |                          |                        |
| High Purity.....        | 5  | 1.0  | 270-310            | 62          | 92          | 100         | 115      | 11                       | 40                     |
| Do.....                 | 5  | 2.5  | 280                | 94          | 99          | 100         | 118      | 12                       | 22                     |
| HP+0.1C.....            | 5  | 2.5  | 330                | 119         | 124         | 124         | 138      | 9                        | 20                     |
| HP+0.25C.....           | 5  | 2.5  | 347                | 132         | 138         | 138         | 150      | 16                       | 27                     |
| HP+0.25C+0.20.....      | 5  | 2.5  | 382                | 142         | 150         | 151         | 159      | 6                        | 5                      |
| HP+0.25C+0.10+0.1N..... | 5  | 2.5  | 401                | 150         | 159         | 160         | 170      | 12                       | 27                     |
| HP+0.25C.....           | 5  | 3.5  | 346                | 121         | 129         | 130         | 143      | 12                       | 28                     |
| HP.....                 | 5  | 5.0  | 313                | 92          | 104         | 106         | 123      | 12                       | 36                     |
| HP+0.25C.....           | 5  | 5.0  | 354                | 127         | 130         | 131         | 142      | 12                       | 28                     |
| HP.....                 | 5  | 10.0 | 372                | 128         | 141         | 146         | 163      | 7                        | 8                      |
| HP.....                 | 5  | 15.0 | 314                | 116         | 128         | 129         | 130      | 7                        | 24                     |
| Commercial.....         | 5  | 2.5  | .....              | 99          | .....       | 133         | 145      | 12                       | 37                     |

The present invention comprises the discovery that desirable structural alloys of the general character of those disclosed in said companion application may be made by the use of chromium, instead of molybdenum, as the ingredient added to a master titanium-base alloy containing a few percent of aluminum.

The present invention comprises the further discovery that, whereas the maximum permissible molybdenum content is somewhat less than 10%, alloys containing as much as 15% of chromium show excellent strength properties and at the same time retain a ductility adequate for structural uses.

The invention comprises the further discovery that the concurrent use of both chromium and molybdenum in a base alloy containing aluminum is productive of high strength alloys of adequate ductility.

The titanium base metal used in the present alloys may contain substances or impurities besides titanium, as normally found in either high purity titanium or commercially pure titanium. It may be, for example, a high purity or "iodide" process titanium, as produced according to the Van Arkel U. S. Patent No. 1,671,213. Alternatively, it may be a commercial titanium, as produced, for example, by magnesium-reduction processes, such as the process of U. S. Patent No. 2,205,854, to Kroll, or modifications thereof; provided that the carbon, oxygen and nitrogen contents of these alloys, hence of the base metal, should not exceed 0.5%, 0.25% and 0.15% respectively, nor should they total more than about 0.5%, if the alloys are to possess good ductility as cast or as worked and annealed.

It has been found, however, that the presence of be-

45 It will be seen that the minimum quantity of chromium which has a material effect is about 1%, that the optimum of chromium is about 2.5%, and that ternary alloys of titanium and aluminum with about 2.5% of chromium are benefited by the addition of carbon, oxygen and nitrogen, in the quantities in which these elements are contained in commercial titanium.

Structurally, after annealing at 850° C., for 3½ hours, the alloys containing 5% chromium show relatively fine 50 equiaxed grains of the alpha phase in a matrix of the beta phase. The alloys of 10% chromium content show a structure of large beta grains containing fine alpha needles in a Widmanstatten pattern. In the 15% chromium alloys the alpha phase has almost disappeared, only a very small amount remaining within the beta grains and 55 along the grain boundaries. As a stabilizer of beta titanium, chromium is more effective than molybdenum.

The alloys of lower chromium content harden as much 60 as 95 Vickers points on quenching from a temperature of 950° C. or higher, while those of higher chromium content may quench soft, this effect being related to the stabilization of beta titanium.

These alloys show excellent resistance to heat softening, and are thus particularly adapted for use at relatively 65 high temperatures. For example, an alloy of 5% aluminum, 2.5% chromium, 0.25% carbon, balance substantially all titanium, having a room temperature hardness of 352 Vickers, shows, at 400° F., a Vickers hardness of 270, and at 600° F., a Vickers hardness of 246. Thus, at 70 600° F., its Vickers hardness has decreased by about 1/3. At 800° F., the Vickers hardness is 226, and at 1000° F., it is 186, a figure comparable with the av-

verage room temperature hardness of commercial titanium.

As above set forth, the optimum chromium content for alloys of this type is about 2.5%. Alloys of comparable properties can be made by substituting molybdenum for part of the chromium. As before, the presence of some carbon, oxygen or nitrogen, is beneficial. Typical alloys of this character, and their properties after hot rolling and annealing at about 850° C., are as follows:

| Composition<br>(Balance<br>Ti) | Annealed<br>Hard-<br>ness | Tensile Properties |                |                |                      |                                     |                              |
|--------------------------------|---------------------------|--------------------|----------------|----------------|----------------------|-------------------------------------|------------------------------|
|                                |                           | Propor.<br>Limit   | 0.1%<br>Offset | 0.2%<br>Offset | Ultimate<br>Strength | Percent<br>Elonga-<br>tion in<br>1" | Percent<br>Area<br>Reduction |
| Al, 5.0                        |                           |                    |                |                |                      |                                     |                              |
| Mo, 1.25                       |                           |                    |                |                |                      |                                     |                              |
| Cr, 1.25                       |                           |                    |                |                |                      |                                     |                              |
| Al, 5.0                        |                           |                    |                |                |                      |                                     |                              |
| Mo, 1.25                       |                           |                    |                |                |                      |                                     |                              |
| Cr, 1.25                       |                           |                    |                |                |                      |                                     |                              |
| C, 0.25                        |                           |                    |                |                |                      |                                     |                              |
| Al, 5.0                        |                           |                    |                |                |                      |                                     |                              |
| Mo, 1.25                       |                           |                    |                |                |                      |                                     |                              |
| Cr, 1.25                       |                           |                    |                |                |                      |                                     |                              |
| C, 0.25                        |                           |                    |                |                |                      |                                     |                              |
| O, 0.1                         |                           |                    |                |                |                      |                                     |                              |
| Al, 5.0                        |                           |                    |                |                |                      |                                     |                              |
| Mo, 1.25                       |                           |                    |                |                |                      |                                     |                              |
| Cr, 1.25                       |                           |                    |                |                |                      |                                     |                              |
| C, 0.25                        |                           |                    |                |                |                      |                                     |                              |
| O, 0.1                         |                           |                    |                |                |                      |                                     |                              |
| N, 0.1                         |                           |                    |                |                |                      |                                     |                              |

These alloys are of the two-phase type, titanium being present in both the alpha and beta forms. Both chromium and molybdenum are within a group of metals which tend to stabilize beta titanium at ordinary temperatures.

The presence of beta titanium in the finished alloy has been found beneficial in increasing both strength and ductility.

In the above table, certain elongation data are missing, due to the fact that rupture occurred at a location such that accurate measurement of elongation was impracticable. Area reduction, however, gives an index of ductility.

The physical properties of these quaternary alloys will be seen to be comparable with, though slightly inferior to, those of the ternary chromium alloys. Structurally, all of the quaternary alloys are similar, consisting of beta particles dispersed intergranularly in a fine grained alpha matrix.

What is claimed is:

1. An alloy containing from about 2% to about 7% aluminum and from about 1% to about 15% chromium, balance titanium.

2. An alloy containing about 5% aluminum and from about 1% to about 15% chromium, balance titanium.

3. An alloy composed essentially of 2% to about 7% aluminum, about 1% to about 15% chromium, and about 0.25% carbon, balance titanium.

4. An alloy composed essentially of about 5% aluminum, about 2.5% chromium, from 0% to about 0.15% nitrogen, from 0% to about 0.25% oxygen, and from 0% to about 0.3% carbon, balance titanium.

5. An alloy composed essentially of about 5% alumi-

num, about 2.5% chromium, about 0.25% carbon, about 0.1% nitrogen and about 0.1% oxygen, balance titanium.

6. An alloy composed essentially of 2%-7% aluminum, 1%-15% chromium, and the balance titanium.

7. An alloy composed essentially of 2%-5% aluminum, 1%-10% chromium, 0.1%-0.3% carbon, and the balance titanium.

8. A ductile titanium base alloy containing: about 2-

30 7% aluminum and about 1-15% chromium, the balance of the alloy being substantially titanium and said alloy being characterized in high resistance to softening at elevated temperatures, and in having an ultimate strength at least 10% in excess of that of the titanium base metal.

35 9. A ductile titanium base alloy containing: about 2-7% aluminum, about 1-15% chromium, up to about 0.15% nitrogen, up to about 0.25% oxygen and up to about 0.3% carbon, the balance of the alloy being substantially titanium and said alloy having an ultimate strength at least 10% in excess of that of the titanium base metal, and being characterized in high resistance to softening at elevated temperatures.

40 10. A titanium base alloy consisting essentially of about: 2 to 7% aluminum and about 1 to 15% chromium, characterized in having an ultimate strength of at least 100,000 p. s. i. and a tensile elongation of at least 2%.

45 11. An alloy consisting of about: 2 to 7% aluminum, 1 to 15% chromium, up to 0.3% carbon, up to 0.25% oxygen, up to 0.15% nitrogen, and the balance titanium.

#### References Cited in the file of this patent

##### FOREIGN PATENTS

571,317 Great Britain ----- Aug. 20, 1945

##### OTHER REFERENCES

"Titanium" Report of Symposium, Dec. 16, 1948, sponsored by Office of Naval Research, pages 108 and 111.

60 U. S. Air Force Project Rand, "Titanium and Titanium-Base Alloys," published by Battelle Memorial Institute, March 15, 1949, pages 11 and 13.